# EUROPEAN PATENT APPLICATION

(11) **EP 0 014 803 A1**
(43) Date of publication of application: **03.09.1980**
(21) Application number: 79302908.3
(22) Date of filing: 14.12.1979
(51) Int. Cl.: D01D 5/253, D01D 5/24, D01F 6/18

(54) **Process for preparing acrylonitrile polymer fiber of hollow or open structure**

(30) Priority: 21.02.1979 US 13342; 21.02.1979 US 13344; 21.02.1979 US 13346; 21.02.1979 US 13353; 21.02.1979 US 13773
(71) Applicant: AMERICAN CYANAMID COMPANY, Wayne New Jersey 06904 (US)
(72) Inventor: Pfeiffer, Ronald E., Pensacola Florida (US); Demaria, Francesco, Gulf Breeze Florida (US); Hamilton, Relmond Harold, Pensacola Florida (US)
(74) Representative: Allam, Peter Clerk

(57) **Abstract**

There is provided a process for preparing acrylonitrile polymer fiber of hollow or open structure which comprises extruding a homogeneous single phase fusion melt of acrylonitrile polymer and waterthrough a spinnerette whose orifices are partially blocked by means of solid inserts, such as strands of wire or removable pins. The fusion melt is extruded directly into a steam-pressurized solidification zone maintained under conditions of saturation, temperature and pressure which control the release of water from the nascent extrudate and maintain the extrudate in a plastic state. While in the solidification zone, the extrudate is stretched to provide orientation of the polymer molecules. The process can provide open and hollow structure acrylonitrile polymer fibers of a wide variety of different cross-sectional shapes while employing spinnerettes which are readily constructed.

## Description

This invention relates to a process for preparing an acrylonitrile polymer fiber of modified cross-sectional shape. More particularly, this invention relates to such a process wherein a single phase fusion melt of acrylonitrile polymer and water is extruded through a spinnerette the orifices of which are partially blocked by solid inserts.

Recent developments in the art of spinning acrylonitrile polymer fiber have led to a fusion melt spinning procedure, see U.S. Patent 4,163,770 issued August 7, 1979, to Harold Porosoff. In this procedure, an acrylonitrile polymer and water in proper proportions are heated to a temperature above the boiling point of water at atmospheric pressure and under sufficient pressure to maintain water in liquid state. At appropriate temperature and pressure a homogeneous fusion melt of polymer and water will form at a temperature below the deterioration temperature of the polymer and at a temperature below which the polymer would normally melt with decomposition. In preferred embodiments, this fusion melt is extruded through a spinnerette directly into a steam-pressurized solidification zone maintained under conditions which prevent sheath-core structure in the cross-section of the nascent filament and enable stretching to provide orientation of the polymer molecules to be accomplished while the extrudate remains within the solidification zone. This proccss provides a rapidly solidified extrudate composition which upon exit from the spinnerette shows n tendency towards stickiness and high conformity to the shape of the spinnerette orifices through which it is spun.

Fibers having hollow or open cross-sectional shape are desirable for a number of reasons. Because of their structure such fibers have a higher extent of surface area than do conventional shaped fibers. This high surface area consists of both external surface area and internal surface area of hollow and open structural modifications. This high surface area permits increased adsorption of water, dyes and other adsorbable materials. Increased water adsorption provides greater comfort in wearing fabrics made from such fiber. The hollow or open structure also provides greater bulk than conventional fiber of the same denier. Esthetic qualities such as handle or feel are also desirably altered by the hollow or open structure and suitable structures can provide greater cover in fabric constructions than conventional structures of the same denier. Fabrics constructed from the open structure fiber dry quicker than fabrics constructed from closed structure fiber because of their greater surface area. Thus, although the desirability of hollow and open structure fibers is generally recognized, suitable processes for preparing such fiber have been difficult to provide and only limited amounts of fiber of hollow and open structures have become available.

Spinnerettes useful in providing hollow and open structure fiber are extremely difficult to construct and require extremely expensive techniques to construct. Spinnerettes useful in one type of fiber-spinning process are not always useful in other types of fiber-spinning processes. Because of these restrictions very limited production of hollow and open structure fiber has been evidenced. This is especially true in the field of acrylonitrile polymer fiber where the previous spinning processes did not respond well to modifications for preparing hollow and open structure fiber. What is needed is a process for spinning hollow and open structure acrylonitrile polymer fiber which employs readily constructed spinnerettes and enables wide variations in the types of modified fiber structure provided. Such a provision would fulfill a long-felt need and constitute a significant advance in the art.

In accordance with the present invention, there is provided a process for preparing acrylonitrile polymer fiber which comprises extruding a homogeneous single phase fusion melt of acrylonitrile polymer and water through a spinnerette directly into a steam-prcssurized solidification zone maintained under conditions of saturation, temperature and pressure which controls the release of water from the nascent extrudate and maintain the extrudate in plastic state and stretching said extrudate while it remains within the solidification zone to provide orientation of the polymer molecules characterized by employing a spinnerette the orifices of which have been partially blocked by means of a solid insert therein whereby hollow or open structure fibers are provided.

The process of the present invention provides acrylonitrile polymer fiber of infinite varieties of hollow and open structures. The spinnerette modifications necessary to provide hollow or open structure fiber is readily accomplished by means of removable solid inserts which partially block part of the orifice volume in accordance with the type of fiber structure desired.

The invention will be described more fully with reference to the accompanying drawings in which Figures 1-4 represent a first embodiment for preparing open structure fiber, Figures 5-9 represent a second embodiment for providing open structure fiber, and.Figures 10-15 represent an embodiment for preparing hollow fibers. More specifically:
Figure 1 represents a cross-sectional view of a portion of a conventional spinnerette showing two adjacent spinning orifices and the counterbores associated therewith as well as top and bottom views thereof;
Figure 2 shows the orifices of Figure 1 modified by insertion of wire therein according to an embodiment of the preseht invention as well as top and bottom views thereof;
Figure 3 shows enlarged bottom views of the spinnerette orifices modified by wire inserts;
Figure 4 represents a photomicrograph of cross--sections of fiber spun according to the present invention using the modified orifices represented by Figure 2;
Figure 5 represents a cross-section of a portion of a spinnerette plate showing a single counterbore and orifice as well as top and bottom views thereof;
Figure 6 represents a side view of a typical insertion pin of the present invention as well as top and bottom views thereof;
Figure 7 represents a cross-section of a single counterbore and orifice with insertion pin positioned therein as well as a top and bottom view thereof;
Figure 8 represents the bottom view of a number of shaped orifices having a variety of shaped pins inserted therein;
Figure 9 represents a photomicrograph of cross--sections spun in accordance with the present invention using the spinnerette modification represented in Figure 7;
Figure 10 represents a cross-section of a portion of a spinnerette plate showing a single counterbore and orifice as well as top and bottom views thereof;
Figure 11 represents a typical insertion pin of the present invention as well as top and bottom views thereof;
Figure 12 represents a cross-section of a single counterbore and orifice with insertion pin therein as well as top and bottom views thereof;
Figure 13 represents the bottom view of a number of shaped orifices having a variety of shaped pins inserted therein;
Figure 14 represents a photomicrograph of cross--sections of fiber spun according to the present invention using the spinnerette modification represented by Figure 12; and
Figure 15 represents a photograph of this hollow fiber and a control fiber with ends submerged in water with dye for tracing.

In carrying out processing to provide the hollow or open structure acrylonitrile polymer fiber in accordance with the present invention, a homogoncous single phase fusion melt of a fiber-forming acrylonitrile polymer and water is prepared in accordance with conventional procedures. This fusion melt is then extruded through a spinncrette assembly which has been modified with solid inserts that block a portion of the orifice volume so as to provide a hollow or open structure in the resulting extrudate. Such extrusion is conducted in such a manner that the extrudate which is in the form of filaments issues directly into a steam--pressurized solidification zone maintained under conditions which prevent formation of a sheath-core structure within the solid polymer area and minimize formation of a density gradient and voids therein. The steam will be maintained under conditions of saturation, temperature and pressure which control the rate of release of water from the nascent extrudate and maintain the extrudate in plastic state. Such conditions are described in the art. While the nascent extrudate remains in the solidification zone, it is subjected to orientation stretching at stretch ratios adequate to provide desirable textile properties in the fiber produced. Such stretching can be accomplished within the steam-pressurized solidification zone because under the steam conditions maintained therein sufficient water remains within the extrudate to maintain the extrudate in plastic state. Stretching may be accomplished in one or more stages while within the solidification zone and can lead to fine denier filaments as well as highly desirable physical properties for textile applications.

The acrylonitrile polymer-water fusion melt when spun through a spinnerette directly into a solidfying medium solidifies rapidly without forming sticky surfaces and retains with high conformity the shape of the orifices without the need for any special provisions such as injection of secondary fluid to retain hollow structure. As a result, a variety of fiber shapes and hollow or open configurations can be employed in producing fiber having excellent conformity to the shape-forming orifices including those providing hollow structures.

In a preferred embodiment of the process of the present invention, a hydrophilic acrylonitrile polymer is employed as the fiber-forming polymer. Such a polymer will contain acrylonitrile units and will have hydrophilic moieties associated therewith. There are other techniques by which hydrophilic moieties can be associated with an acrylonitrile polymer.

One method of introducing hydrophilic units into an acrylonitrile polymer composition is to copolymerize acrylonitrile with a hydrophilic comonomer, to provide a copolymer containing at least 50 weight percent of acrylonitrile units, from 1 to 10 weight percent of a hydrophilic monomer and any balance of one or more monomers copolymerizable with acrylonitrile. Another method is to polymerize the acrylonitrile polymer composition in the presence of a redox initiator system that introduces acid groups at the polymer chain ends. Yet another method is to polymerize the acrylonitrile polymer composition in the presence of a pre-formed hydrophilic polymer such as polyvinyl alcohol. Still another method is to hydrolyze a small portion of the acrylonitrile units of a pre-formed acrylonitrile polymer to provide hydrophilic acrylic acid and/or acrylamide units. Further, one can modify a portion of the acrylonitrile units of a pre-formed acrylonitrile polymer by suitable reaction to provide hydrophilic groups, such as by reaction with ethylenediamine to provide imidazoline units. These and other methods known to those skilled in the art can be used alone or in combination to provide hydrophilic units associated with the acrylonitrile polymer composition used to prepare the fiber of the present invention.

An acrylonitrile polymer composition useful to provide the fiber in accordance with the invention may by a single polymer or a blend of compatible polymers so long as the composition provides a minimum of at least 50 weight percent acrylonitrile units and preferably has hydrophilic units associated therewith to achieve a transparent fiber. This transparency is reflected in a dye intensity of at least 60 and a shade change due to hot-wet processing of less than 25. Dye intensity is the reflectance of a dyed fiber of the present invention relative to the reflectance of a wet--spun fiber of the same polymer dyed with the same amount of the same dye. Shade change due to hot-wet processing is the change in reflectance of the dyed fiber after a hot-wet processing step, such as oven drying the wet dyed fiber, compared to the air dried dyed fiber. Individual compatible polymers in blends used need not contain the specified amounts of acrylonitrile units or hydrophilic moieties so long as the total blend composition provides the required amounts of such materials. By hydrophilic moieties are meant those portions of the acrylonitrile polymer composition that are hydrophilic and include such moieties as sulfonic acid groups, polyvinyl alcohol segments, repeating comonomer units and the like. By associated therewith is meant that such hydrophilic units are present in the acrylonitrile polymer composition in a manner appropriate for the particular hydrophilic moieties involved. Thus, sulfonic acid groups may arise as end groups on polymer chains or as a functional group on a comonomer; polyvinyl alcohol moieties may be present as part of a grafted polymer; other hydrophilic moieties may arise as repeating units in a copolymer prepared from two or more monomers or as a result of hydrolyzing a suitable polymer; they may also arise as a result of suitable reaction of a pre-formed polymer; they may arise as a compatible polymer blend; and in such other methods as are known to those skilled in the art. Thus, the term associated therewith is intended to include the various manners in which hydrophilic moieties are present in the acrylonitrile polymer composition since no other terminology is appropriate to cover all the manners described.

The amount of hydrophilic moieties in a given acrylonitrile composition will vary depending upon many factors. The content of hydrophilic moieties will be influenced by the nature of the hydrophilic groups, the molecular weight of the polymer, the content of acrylonitrile in the polymer, the nature of the polymer composition, i.e. copolymer, graft, blend, etc., the presence or absence of more than one type of hydrophilic moieties, processing conditions and other variables. Generally useful amounts of hydrophilic moieties are those which as monomer units comprise about 1 to 10 weight percent of the total polymer weight. However, useful contents of hydrophilic moieties can readily be found by trial following the teachings herein as a guide.

Suitable acrylonitrile polymers include homopolymers of acrylonitrile and copolymers of acrylonitrile and one or more of the following monomers.

### HYDROPHOBIC MONOMERS

Methyl acrylate, ethyl acrylate, butyl acrylate, methoxymethyl acrylate, beta-chloroethyl acrylate and the corresponding esters of methacrylic acid and chloro-acrylic acid; vinyl chloride, vinyl fluoride, vinyl bromide, vinylidene chloride, vinylidene bromide, allyl chloride, l-chloro-l--bromoethylene; methacrylonitrile, methyl vinyl ketone, vinyl formate, vinyl acetate, vinyl propionate, vinyl stearate, vinyl benzoate, N-vinyl phthalimide, N-vinyl succinimide, methylene malonic esters, itaconic esters, N-vinyl carbazole, vinyl furan, alkyl vinyl ethers, diethyl citraconate, dimethyl mesaconate, styrene, dibromostyrene, vinyl naphthalene, 2-methyl-l-vinyl imidazole, 4-methyl-l-vinyl imidazole, 5-methyl-l-vinylimidazole and the like.

### HYDROPHILIC MONOMERS

Acrylic acid, methacrylic acid, alpha-chloroacrylic acid, itaconic acid, vinyl sulfonic acid, styrene sulfonic acid, methallyl sulfonic acid, p-methoxyallyl benzene sulfonic acid, acrylamidomethylpropane sulfonic acid, ethylene-α,β--dicarboxylic acids and their salts; acrylamide, methacrylamide, dimethyl acrylamide, isopropyl acrylamide; allyl alcohol; 2-vinyl pyridine, 4-vinylpyridine, 2-methyl-5-vinylpyridine; vinylpyrrolidone; vinyl piperidone; 1,2-dihydroxypropyl methacrylate, hydroxyethyl methacrylate; 1-trimethylammonium--2-hydroxypropyl methacrylate methosulfate; and the like.

In preparing acrylonitrile polymers and copolymers it is desirable to employ redox systems such as sodium per- persulfate-sodium bisulfite to initiate and control the polymerization. Such use results in sulfonic acid end groups on the polymer formed. The proportion of sulfonic acid end groups in the polymer will vary with molecular weight of the polymer, higher proportions being present in polymers of low molecular weight. These sulfonic acid end groups should be taken into account when determining the content of hydrophilic moieties in the acrylonitrile polymer composition used to provide the fiber in accordance with the present invention. Acrylonitrile polymer compositions containing sulfonic acid groups arising solely from the use of an appropriate redox system can be effectively employed to provide fiber in accordance with the present invention. When hydrophilic pre-formad polymers such as polyvinyl alcohol, polyvinyl pyrrolidone, polyethylene oxide, polyacrylamide, polyacrylic acid and the like are to be used to provide the acrylonitrile polymer composition, it is desirable that such pre-formed be added to the monomer composition to be polymerized to provide the acrylonitrile units. Individual polymers of the composition may range in molecular weight from about 10,000 to 200,000 or more so long as the composition provides fiber of desirable properties.

Once a desired acrylonitrile polymer composition for forming fiber has been selected, it is next necessary to prepare a single phase homogeneous fusion melt of the composition and water. A single phase fusion melt of acrylonitrile polymer composition and water results when suitable quantities of polymer composition and water are heated at elevated temperature and pressure sufficient to maintain water in liquid state. The amount of water necessary will vary depending upon the polymer composition employed. For a given polymer composition, there will be a range of water contents that will provide the single phase fusion melt at the operating temperature and pressure. This can readily be determined from a phase diagram, which will also indicate the minimum melt temperature, i.e. the temperature at which the polymer begins to melt. Use of too low a water content or temperature will result in a separate phase of unmelted polymer. Use of too high a water content will result in a separate phase of polymer-water melt and an added phase of free water. Usually effective amounts of water are in the range of about 5-35 weight percent based on the total weight of polymer and water. When a hydrophilic polymer composition is employed, it is generally preferable to use a water content in the lower half of this range, i.e. about 5 to 20 weight percent. The fusion melt should be obtained at a temperature safely below the deterioration or decomposition temperature of the polymer composition. Sufficient temperature and mixing should be employed to ensure that a homogeneous fusion melt is obtained. Useful temperatures are generally in the range of about 140-200°C.

The fusion melt is conveniently obtained in conjunction with spinning using a screw extruder coupled with a pump - and spinnerette. A suitable procedure for melt spinning is described in U.S. Patent 3,991,153 issued November 9, 1976 to G. K. Klausner et al. Other types of melt-spinning devices may be used such as a piston pump in conjunction with a spinnerette.

In carrying out processing in accordance with the present invention, the homogeneous single phase fusion melt of acrylonitrile polymer composition and water is extruded througli a spinnetette directly into a steam-pressurized solidification zone maintained under conditions of saturation, temperature and pressure which control the release of water from the nascent extrudate and maintain the extrudate in plastic state. Under these conditions the extrudate is solidified and remains in a state such that orientation stretching can be accomplished while the extrudate remains in the solidification zone. Usually the solidification zone is pressurized with saturated steam at a temperature which is about 10 to 30°C. below the minimum melt temperature of the polymer-water composition. As the stretched extrudate emerges from the solidification zone, it enters atmospheric conditions. When the extrudate enters the atmosphere, required processing according to the present invention is complete but such additional conventional processing as may be desired can be performed.

A preferred added processing stop in instances where a hydrophilic polymer composition is cmployed is to dry the extrudate in an oven under conditions specified by dry--bulb and wet-bulb temperatures. Generally, the dry-bulb will be in the range of 120-180°C. and the wet-bulb will be in the range of 60-100°C. This drying step is preferably conducted before any uncontrolled or tensionless shrinkage of the extrudate has occurred. This drying step may be conducted on the extrudate in a frec-to-shrink condition or under tension.

Another preferred subsequent processing step is that of relaxing the extrudate in steam under pressure so as to achieve shrinkage of about 5-40%. This relaxing step should follow the drying step when such drying is effected.

In order to obtain the open structure or hollow cross-section in the resulting fiber, fit is necessary to employ a spinnerette that has orifices that will provide the desired configurations. A desirable procedure to obtain useful spinnerettes is to modify a conventional spinnerette plate as will next described.

The conventional spinnerette plate will contain a plurality of orifices and each orifice will have a counterbore to enable operative back pressure to be achieved. Such spinnerettes should be of a material of construction, useful in melt spinning applications.

In one embodiment for providing fiber of open structure, wire is inserted into the brifices of the spinnerette orifices to block a suitable portion thereof and contact the orifice surface at some point. Wire of suitable-construction material and size is provided for insertion to provide the orifice modification desired. A number of techniques for providing the wire modification of the orifices is possible. In one procedure, a single strand of suitable wire can be passed alternatively up and down through adjacent orifices until all orifices are modified and the wire ends are joined to secure the wire in position. Alternatively, such technique could be used in modifying with one wire strand only the orifices in one orifice row or in modifying only two adjacent orifices. Another technique involves providing the wire in pre-cut and pre-shaped sections which then can be inserted through the counterbores to modify adjacent orifices while providing a secure fit. It is also possible to use more than one wire to block portions of one orifice and suitable securing procedures can involve multiple wires. Additional methods of securing the wires are possible and will readily occur to those skilled in the art.

The wires used to block a part of the spinnerette orifice may be of different size and shape depending upon the nature of blocking and the resulting fiber cross-section desired. The wire, of course, should be of suitable size to fit within the orifice and leave sufficient opening for operability of the fiber spinning process. Wire of round cross-section is most common and is useful for many desirable modifications of fiber cross-section. Additional shapes of useful wire cross-sections include triangular, square, rectangular, elliptical, hexagonal, and the like as well as irregular shapes. Additional variations arise from use of orifices of cross--sectional shapes other than round and placing different shaped wires therein. Combinations of several different shaped wires in an appropriate shaped orifice can lead to unusual fiber cross-sections providing maximization of those desirable properties for which shaped fiber cross-sections are desired.

A preferred embodiment of the process of the present invention is shown with respect to Figures 1-4. Figure 1 represents a cross-sectional view of a portion of a conventional spinnerette plate showing two adjacent orifices and the countcr- bores associated therewith as well as top and bottom views of the orifices. Figure 2 represents the same view as Figure 1 except that the orifices have been modified with wire in accordance with the present invention. In this embodiment, a round cross-section wire was employed which was bent to modify two orifices and was inserted in a manner in which the wire touches the wall of the orifice so as to provide an open-structure fiber cross-section. Spring tension in the bent wire keeps it securely placed in the two orifices. Figure 3 shows enlarged boctom views of the modified orifices and Figure 4 shows the crescent-shaped cross-sections of the fiber obtained.

Another procedure for obtaining the open structure fiber cross-sections is by the insertion of pins in the counterbore-orifice combination of a conventional spinnerette plate. These pins are designed so that they are of solid construction and occupy a fixed position within the counterbore. The pins will be of such size as to enable extrusion composition to flow through the counterbores at operative back pressure to the orifice. The pins will typically have an upper portion which fits into the counterbore and a lower portion which fits into the orifice. The upper portion will be of suitable dimensions to assume a fixed position within the counterbore so that the lower portion remains suitably disposed in the orifice to provide the open structure fiber and enable adequate flow of extrusion composition through the counterbore and capillary. The lower portion of the pin will be of suitable dimensions to fit within the orifice and contact a portion of the wall thereof while providing a desirable relationship between fiber wall and open structure therein.

A preferred embodiment of this type of modification is shown with reference to Figures 5, 6 and 7. Figure 5 represents a cross-section of a typical counterbore-orifice combination used in a typical spinnerette plate, as well as top and bottom views thereof. The counterbore has a greatly enlarged diameter relative to that of the orifice and converges to the orifice diameter with proper sloping. Figure 6 represents a side view of a preferred pin insert to provide open structure fibers when inserted within the counterbore-capillary combination as well as top and bottom views thereof. As can be seen, the upper portion of the pin resembles a cylindrical rod which has been flattened along its length to provide clearance on two sides with the counterbore. The top of the upper portion is leveled while the bottom thereof is tapered _{'}at a greater angle than the taper of the counterbore to connect the orifice and thus provides clearance for the extrusion material. The bottom portion of the pin has a solid crcss--sectional shape that conforms to the shape of the orifice on one face which is positioned so as to contact a portion of the wall of the orifice and has additional shape to provide desirable open area within the extrudate issuing from the orifice and provide suitable fiber cross-sectional structure. In Figure 7, the insertion of the pin of Figure 6 in the counterbore-capillary combination of Figure 5 is shown in cross-section along with top and bottom views thereof. Clearance of the pin from the counterbore wall is shown in the top view and clearance between the tapers of the pin and counterbore are shown in the cross-section. In the bottom view the space in the orifice occupied by the pin insert is shown and the resulting cross-sectional shape of the extrudate can be seen.

In Figure 8 is shown a variety of orifice shapes with various shapes of the lower portion of the insert pin that can be used in the process of the invention. As can be seen, the pin shape may vary widely as may the orifice shape. Also, it is possible to provide one or more open areas within the fiber by use of multiple projections as the lower portion of the pin insert.

Figure 9 shows cross-sections of fiber obtained by the process of the invention using in the counterbore-capillary combinations pin inserts as shown in Figure 7.

To provide hollow fibers, pin inserts resembling those described above are used except that the lower portion of the insert pin is centered in the orifice and does not contact the orifice wall. This is illustrated in Figures 10-15. Figure 10 represents a cross-section of a typical counterbore--capillary combination as well as top and bottom views thereof. Figure 11 represents a side view of a preferred pin insert to provide hollow fibers when inserted within the counterbore--capillary combination as well as top and bottom views thereof. The upper portion of the pin insert is to that of Figure G. The lower portion is similar to that of Figure 6 but is centered and does not have conformity to the orifice wall since it does not contact such wall. In Figure 12 the insertion of the pin of Figure 11 in the counterbore-capillary combination of Figure 10 is shown in cross-section along with top and bottom views thereof. Clearance of the pin from the counterbore wall is shown in the top view and clearance between the tapers of the pin and counterbore are shown in the cross-section. In the bottom view the space between the two inner circles represents the wall thickness of the extrudate as spun.

In Figure 13 is shown a variety of orifice shape with various shapes of the lower portion of the insert pin that can be used in providing hollow fibers. As can be seen the pin shape can vary widely as well as can the orifice shape. Also, it is possible to provide one or more hollows within the fiber by use of multiple projections as the lower portion of the pin insert.

Figure 14 represents a photomicrograph of fibers spun by the process of the invention using the pin modification shown in Figure 12, showing the hollow structure of fiber ends.

Figure 15 shows the greater wicking tendencies of hollow fibers comparied to solid fibers.

The invention is more fully illustrated in the examples which follow wherein all parts and percentages are by weight unless otherwise specified.

### EXAMPLE 1

A conventional spinnerette plate having a plurality of orifices of 200 micron diameter was modified as shown in Figure 2 with 150 micron diameter wire resulting in free area remaining in the individual holes of about T3, 740 square microns. Modification was effected by cutting short lengths of the wire, about 1 inch, and feeding the ends through adjacent orifices from the counterbore side. The wire was then pulled tight which conformed the wire to the counterbore, cut to approximate length and filed to fit flush to the capillary exit.

An acrylonitrile polymer of the following composition was employed:
Onto a pre-formed polyvinyl alcohol (Elvanol 71-306) was grafted suitable components to provide a polymer composition of:

The polymer had a kinematic molecular weight of 42,000. Kinematic molecular weight (M̅_{K}) is obtained from the relation- ship/κ=1/A M̅_{K} wherein is the average effluent time in seconds for a solution of 1 gram of the polymer in 100 milliliters of 50 weight percent aqueous sodium thiocyanate solvent at 40°C. multiplied by the viscometer factor and A is the solution factor derived from a polymer of known molecular weight.

The polymer, 86 parts, and water, 14 parts, were prepared as a fusion melt in an extruder at 160°C. and autogenous pressure and extruded through a spinnerette plate prepared as described above. Extrusion was directly into a steam-pressurized solidification chamber maintained at 13 pounds per square inch gauge with saturated steam and stretching was accomplished in the solidification chamber at a stretch ratio of 3.1 in a first stage and 8.3 in a second stage for a total stretch ratio of 25.7. The resulting fiber of about 5 denier per filament had a cross-sectional shape as shown in Figure 4, which shape is termed crescent-shaped.

### EXAMPLE 2

A conventional spinnerette plate having a plurality of orifices of 200 micron diameter was fitted with insert pins as shown in Figure 7. Each pin was 175 microns in diameter resulting in free area remaining in the individual capillaries of about 7,363 square microns.

The acrylonitrile polymer composition described in Example 1 was employed.

A mixture of 83 parts of the polymer, 17 parts water and 0.25 parts of a conventional glycol stearate type lubricant was converted into a fusion melt in an extruder at 175°C. and autogenous pressure and extruded through the . spinnerette plate modified as described above. Extrusion was directly into a steam-pressurized solidification chamber maintained at 11 pounds per square inch gauge with saturated steam. The filaments were stretched at a stretch ratio of 3 while in the solidification zone to give a fiber of about ₄0 denier per filament that had cross-sectional shape as shown in Figure 9 which shape is termed crescent-shaped.

### EXAMPLE 3

A conventional spinnerette plate having a plurality of orifices of 300 micron diameter was fitted with insert pins as shown in Figure 12. Each pin was 175 micron in diameter resulting in free area remaining in the individual capillaries of about 46,633 square microns.

Acrylonitrile polymer of the composition of that of Example 1 but of kinematic molecular weight of 40,000 was employed.

A mixture of 84.6 parts polymer, 15.4 parts water and 0.25 parts of a conventional glycol stearate type lubricant was converted to a fusion melt in an extruder at 167°C. and autogenous pressure and.extruded through the spinnerette plate prepared as described above directly into a steam--pressurized solidification chamber maintained at 13 pounds per square inch gauge with saturated steam. The resulting filaments were stretched while in the solidification chamber at a stretch ratio of 9.2 in a first stage and 6.4 in a second stage of give a fiber of about 6.5 denier per filament. The fiber was dried at 139°C. dry-bulb and 74°C. wet-bulb and steam-relaxed at 116°C. The final denier fiber obtained was hollow as shown in Figure 14.

When ends of this fiber were submerged in water containing dye, water wicks up above the water surface for 4 inches. When ends of a comparable solid fiber were submerged in the same dye-water composition, no wicking was observed. This is shown in Figure 15.

## Claims

1. A process for preparing acrylonitrile polymer fiber which comprises extruding a homogeneous single phase fusion melt of acrylonitrile polymer and water through a spinnerette directly into a steam-pressurized solidification zone maintained under conditions of saturation, temperature and pressure which control the release of water from the nascent extrudate and maintain the extrudate in plastic state and stretching said extrudate while it remains within the solidification zone to provide orientation of the polymer molecules characterized by employing a spinnerette the orifices of which are partially blocked by means of a solid insert therein whereby hollow or open structure fibers are provided

2. The process of Claim 1 further characterized by use of a hydrophilic acrylonitrile polymer and drying the stretched extrudate at conditions represented by dry-bulb temperatures in the range of 120°-180°C and wet-bulb temperatures in the range of 60°-100°C.

3. The process of Claim 1 or Claim 2, wherein the stretched extrudate is relaxed in steam under pressure.

4. The process of preceding claim, wherein said insert provides a fiber having a shaped cross-sectional structure comprising a contigous solid polymer area and associated therewith an open area, said solid polymer area extending continuously along the entire length of the fiber and forming an outer surface thereon, said open area also extending continuously along the entire length of the fiber and providing an inner surface therein, and said inner surface communicating with said outer surface and providing at least 1/3rd as much surface as said outer surface.

5. The process of Claim 4, wherein said polymer area is crescent-shaped.

6. The process of any preceding claim, wherein each said insert is a strand of wire positioned within a spinnerette orifice so as to touch the wall thereof.

7. The process of any one of Claims 1-4, wherein said spinnerette contains a plurality of orifices with a counterbore for each orifice and wherein each said solid insert is a removable pin positioned within its orifice to have an upper portion located within the counterbore thereof and a lower portion located within the orifice, said upper portion occupying a fixed position within said counterbore and enabling spinning composition to flow through the counterbore to the orifice at operative back pressure and said lower portion contacting a portion of the wall of the orifice to provide an open structure extrudate.

8. The process of any one of Claims 1-3, wherein said insert provides a hollow fiber.

9. The process of Claim 8, wherein said spinnerette contains a plurality of orifices with a counterbore for each orifice, and wherein each said solid insert is a removable pin positioned within its orifice to have an upper portion located within the counterbore thereof and a lower portion located within the orifice, said upper portion occupying a fixed position within said counterbore and enabling spinning composition to flow through the counterbore to the orifice at operative back pressure, and said lower portion being spaced from the orifice wall to provide a hollow extrudate.
